

# UNITED STATES PATENT OFFICE

1,994,275

## BIMETALLIC ARTICLE

Herbert W. Graham and Samuel L. Case, Pittsburgh, Pa., assignors to Jones & Laughlin Steel Corporation, Pittsburgh, Pa., a corporation of Pennsylvania

No Drawing. Application March 16, 1933,  
Serial No. 661,891

1 Claim. (CL 29—181)

This invention relates to bimetallic bodies and particularly to bodies having a ferrous base and a coating of zinc. The use of zinc in hot galvanizing to protect steel is well known. The character of the zinc coating is always a matter of concern to the manufacturer and requires the closest control and inspection. It is desirable to obtain a tightly adherent coating which will not peel or flake, and various schemes for improving the character of the coating have been proposed.

We have found that the quality of the coating may be vastly increased by alloying the zinc with a small amount of metallic sodium. We have found that 2% of sodium is about the maximum which can be alloyed with the zinc, but this small percentage fundamentally affects its properties. It makes the metal more dense and

imparts a finer structure. Sheets or wires coated with this zinc-sodium alloy are superior to the ordinary galvanized coating.

We have described a present preferred embodiment of our invention. It will be understood, however, that this is by way of illustration only and that it may be otherwise embodied or practiced within the scope of the following claim.

We claim:

As a new manufacture, a bimetallic body comprising a ferrous base having a tightly adherent coating in direct contact with the base, the coating being a binary zinc-sodium alloy, the sodium being present in amounts up to 2%.

10

15

HERBERT W. GRAHAM.  
SAMUEL L. CASE.